

# UNITED STATES PATENT OFFICE.

VICTOR J. KUESS, OF TUNIS, TUNIS.

## ARTIFICIAL FUEL AND PROCESS OF MAKING THE SAME.

No. 830,333.

Specification of Letters Patent.

Patented Sept. 4, 1906.

Application filed March 1, 1904. Serial No. 196,080.

*To all whom it may concern:*

Be it known that I, VICTOR JOSEPH KUESS, a citizen of the Republic of France, and a resident of No. 2 Rue Gharnouta, Tunis, Tunis, 5 have invented a certain new and useful Artificial Fuel and Process of Making the Same; and I do hereby declare the following to be a full, clear, and exact description of the invention, such as will enable others skilled in the 10 art to which it appertains to make and use the same.

This invention relates to a process for solidifying petroleum and other mineral oils for use as fuel.

15 The quantitative proportions of substances to be employed in producing an agglomerated mass or cake of fuel varies according to the quantity of petroleum or mineral to be converted. For facility of explanation suppose that it is desired to solidify petroleum weighing eight hundred grams per liter. For one hundred liters of petroleum reduce to fine division ten kilos of dark rosin, resin or any other hydrocarbon of the turpentine series. Dissolve the resin cold in the petroleum by constant stirring. First melt separately ten kilos of beef suet or any other animal fat, and when the tallow is quite liquefied pour it into the mixture (petroleum 20 and resin) and stir thoroughly. Leave it to cool, stirring it from time to time. Also separately dissolve five kilos of caustic soda in ten liters of water and add the solution to the mass, at the same time stirring. After about 25 two hours add, pouring in a little at a time, a liter of hydrochloric acid. The mass will become hot and liquefy, and the various substances will become intimately combined with the petroleum. Then dissolve two 30 kilos of caustic soda in five liters of water, and after about four hours pour into the mass this new solution while stirring. Leave the pasty product for two or three days. At the end of that time melt the mass on a slow fire and immediately withdraw it from the fire and leave it to cool. If it is desired to use simple solidified petroleum, redissolve it in ten liters of water and pour the solution in molds or shapes. If, on the contrary, it is desired to 35 make briquets for heating purposes to burn less quickly than petroleum, simply melt the solidified petroleum formed as above indicated and add a certain quantity of water. The water will be completely incorporated. 40 Withdraw the mass from the fire, still liquid 45

and hot, and mix with it other solid combustibles reduced to a fine state of division—for example, sawdust, coal-dust, wood-carbon, lignite finely crushed, bark, or other such divided substances. Moreover, the more one 50 adds of these combustible substances to the petroleum base the more slowly will the briquets burn.

Excellent briquets can be made by adding to ten kilos of solidified petroleum two 55 liters of water and stirring intimately into the boiling mass six kilos of oak sawdust. One obtains thus masses which when compressed form briquets of very firm character, giving a bright flame, burning without 60 smell, making only little smoke, and above all generating a very intense heat—to wit, about fourteen thousand five hundred calories.

Calorimetric tests of my fuel in comparison 70 with the other commercial fuels have given the following results: wood, six thousand calories; coal, seven thousand two hundred calories; charcoal, eight thousand calories; petroleum, twelve thousand calories; Kuess's 80 fuel, fourteen thousand five hundred calories. The product obtained by me dissolves completely in water without leaving any floating greasy or oily substance. Upon melting the product and boiling it the petroleum does not 85 separate, and upon recooling the briquet becomes uniformly solid again and without a trace of separation. When the product is dissolved in water and precipitated with hydrochloric acid, three distinct fatty bodies are 90 obtained, of which bodies two are soluble in sulfuric acid. The third body, a liquid, is apparently a form of petroleum which is completely soluble in concentrated sulfuric acid.

In one experiment made by me the petroleum 95 employed as an ingredient of the artificial fuel gave the reading "25" on the polariscope, while the new hydrocarbon, separated out by analysis, as above explained, gave the reading "30." Moreover, the petroleum as 100 used was laevo-rotatory, whereas the new hydrocarbon was dextro-rotatory, thus showing that it is no longer possible to recover the original petroleum by analysis and establishing the fact that the petroleum has become 105 chemically bound in the fuel to the extent that it cannot afterward be segregated by any physical treatment.

I claim—

1. In the manufacture of artificial fuel, the 110

process of solidifying mineral oil, which consists in dissolving resin and animal fat in the mineral oil, then acting on the mixture with an alkali and then adding an acid to the resultant mixture.

2. In the manufacture of artificial fuel, the process of solidifying mineral oil, which consists in dissolving resin and animal fat in the mineral oil, then acting on the mixture with 10 an alkali, and then adding hydrochloric acid to the resultant mixture.

3. In the manufacture of artificial fuel, the process of solidifying mineral oil, which consists in dissolving resin and animal oil in the 15 mineral oil, then acting on the mixture with caustic soda, and then adding an acid to the resultant product.

4. In the manufacture of artificial fuel, the process of solidifying mineral oil, which consists in dissolving resin and animal fat in the 20 mineral oil, then acting on the mixture with caustic soda, and then adding an acid to the resultant product.

5. In the manufacture of artificial fuel, the process of solidifying mineral oil, which consists in dissolving a hydrocarbon of the terpene series and an animal fat in the mineral oil, then acting on the mixture with an alkali, 25

and then adding an acid to the resultant product.

6. The process which consists in adding ten kilos of resin and ten kilos of animal fat to one hundred liters of petroleum, then adding to the mixture a solution of five kilos of caustic soda in ten liters of water, and then 30 35 adding one liter of hydrochloric acid to the resultant compound.

7. In the manufacture of artificial fuel, the process which consists in dissolving a hydrocarbon of the terpene series and an animal fat in mineral oil, then acting on the mixture with an alkali, then adding an acid to the resultant product, and then mixing the mass thus obtained with a comminuted solid combustible material. 40

8. An artificial fuel containing chemically-bound mineral oil.

9. An artificial fuel containing chemically-bound mineral oil and a comminuted solid combustible material. 50

In witness whereof I have hereunto set my hand in presence of two witnesses.

V. J. KUESS.

Witnesses:

P. JULLVIERY,  
N. RALLY.